

[54] ARRANGEMENT FOR A SHADOW MASK IN  
A SLIM COLOR TELEVISION TUBE AND  
THERMOSTAT METAL FOR USE THEREIN

[75] Inventor: Jacob L. Ornstein, Norton, Mass.

[73] Assignee: Texas Instruments Incorporated,  
Dallas, Tex.

[22] Filed: Aug. 7, 1972

[21] Appl. No.: 278,335

[52] U.S. Cl..... 313/85 S, 29/195.5, 313/92 B

[51] Int. Cl..... H01j 29/06

[58] Field of Search..... 313/85 S, 92 B

[56] References Cited

UNITED STATES PATENTS

|           |         |               |          |
|-----------|---------|---------------|----------|
| 3,330,980 | 7/1967  | Shrader ..... | 313/85 S |
| 3,524,973 | 8/1970  | Rigdon .....  | 313/85 S |
| 3,617,787 | 11/1971 | Plukker ..... | 313/85 S |
| 3,639,798 | 2/1972  | Miller .....  | 313/85 S |

Primary Examiner—Roy Lake  
Assistant Examiner—Siegfried H. Grimm  
Attorney—Harold Levine et al.

[57] ABSTRACT

A support arrangement for the shadow mask in a color television tube of slim design is shown to include a plurality of support members formed of a low cost thermostat metal embodying only iron alloy materials, which thermostat metal displays high strength and corrosion resistance at elevated temperatures and displays low flexibility and stable thermal response properties, the thermostat metal having outer metal layers of approximately equal thickness formed of nickel-chromium-iron and nickel-iron alloys respectively and having an intermediate layer of a selected stainless steel comprising between 45 and 65 percent of the total thickness of the thermostat metal providing the thermostat metal with a flexibility in the range from 90 to 110 in the temperature range from room temperature up to about 350°F.

1 Claim, 3 Drawing Figures



PATENTED DEC 25 1973

3,781,583

SHEET 1 OF 2



Fig. 1.

PATENTED DEC 25 1973

3,781,583

SHEET 2 OF 2



Fig. 2.



Fig. 3.

**ARRANGEMENT FOR A SHADOW MASK IN A SLIM COLOR TELEVISION TUBE AND THERMOSTAT METAL FOR USE THEREIN**

In a color television tube wherein electron source means within the tube direct electrons onto phosphors located on the inner surface of the tube face, it is customary to mount a shadow mask having a very large number of very small holes between the electron source means and the tube face so that only electrons following selected paths are permitted to pass through the mask openings to strike respective phosphors. As these shadow masks tend to become heated and tend to expand during tube operation, it has also been customary to mount the shadow mask on the tube envelope by use of thermostat metal support members which move the mask toward the tube face as the mask is heated to compensate for the thermal expansion of the mask to retain proper registration of the mask apertures with respective phosphors on the tube face. Where these thermostat metal members are located inside the tube envelope, it is important that the thermostat metal material be free of any tendency to corrode or to contaminate the tube atmosphere or phosphors during heating thereof; the thermostat metal material must be of relatively high strength at elevated temperatures to support the shadow mask throughout a long tube life; and the thermostat metal material must retain its thermal response characteristics for a long period of time while undergoing repeated heating and cooling. As iron alloy materials have displayed these desirable characteristics for use inside the tube envelopes, it is desirable that the thermostat metals be formed of such iron alloys.

Most recently, with the advent of the slim color television tube having a relatively short space between the tube face and the electron source means within the tube, it is found that only very small shadow mask movement is required or can be permitted for retaining registration of the shadow mask apertures within respective tube face phosphors during thermal expansion of the mask and it is found that the thermostat metal materials customarily used in shadow mask supports have tended to display excessive flexibility making it difficult to proportion shadow mask supports to provide the required compensation for thermal expansion of the mask.

It is an object of this invention to provide a novel and improved support arrangement for the shadow mask in a slim color television tube; to provide such a support arrangement utilizing novel and improved thermostat metal material; to provide such improved thermostat metal material embodying iron alloy material layers which displays high strength and corrosion resistance at relatively high temperatures and which retains its thermal response characteristics throughout a long cycle life; to provide such thermostat metal material which displays low flexibility in temperature ranges from room temperature up to about 350°F.; and to provide such thermostat metal material which is characterized by low cost.

Other objects, advantages and details of the shadow mask support arrangement and thermostat metal of this invention appear in the following detailed description of preferred embodiments of the invention, the detailed description referring to the drawings in which:

FIG. 1 is a plan elevation view of a color television tube partially in section illustrating the shadow mask support arrangement provided by this invention.

FIG. 2 is a plan elevation view to enlarged scale of a thermostat metal support member utilized in the support arrangement of FIG. 1; and

FIG. 3 is a front elevation view of the support member shown in FIG. 2.

Referring to the drawings, 10 in FIG. 1 illustrates a 10 conventional, slim color television tube incorporating the support arrangement for a shadow mask as provided by this invention. As the tube 10 is of conventional structure except for the shadow mask support arrangement, the tube is only partly illustrated in FIG. 1 to show the tube envelope 12, electron source means 14, the tube face 16 having color phosphors 18 thereon, bosses 20 integrally formed on the tube envelope, and a shadow mask 22. As will be understood, the phosphors 18 are arranged in a multiplicity of groups 15 of three colors on the tube face 16 and the shadow mask comprises a sheet of metal such as a sheet of steel foil about 0.005 inches thick having a multiplicity of holes about 400,000 in number (not shown) registered with respective phosphors 18 on the tube face so that 20 only electrons following selected paths from the source means 14 are permitted to pass through the mask apertures to strike respective phosphors 18. The shadow mask apertures are arranged in a conventional pattern over the effective area of the shadow mask which subtends an angle  $\alpha$  from the electron source means 14 of about 110° as illustrated in FIG. 1. In this regard, when a color television tube is hereinafter described as being of slim design, it will be understood that the effective area of the shadow mask of the tube subtends an angle 25 of at least about 110° from the electron source in the tube. As will be understood, the tube 10 is adapted to become heated during operation, this heating resulting in thermal expansion of the shadow mask 22.

40 In accordance with this invention, the shadow mask 22 is supported between the electron source means 14 and the tube face 16 by a plurality of support members 24 (only two of which are shown in FIG. 1) for registering the shadow mask apertures with the respective phosphors 18 on the tube face 16, these support members 24 each being formed of a three-layer composite thermostat metal. Typically, for example, each of the support members 24 has a curved hinge-like portion 26 and two flange portions 28 and 30 extending therefrom, the flange 28 having two apertures 32 fitted over matching bosses 20 on the tube envelope 12 and the flange 30 being welded or otherwise fixedly secured to the shadow mask 22 in any conventional manner.

45 In accordance with this invention, each of the thermostat metal support members 24 is formed of a novel and improved thermostat metal material particularly adapted for supporting the shadow mask 22 in a color television tube 10 of slim design. That is, the support members 24 are each formed of a composite metal laminate having one outer layer 34 and another outer layer 36 metallurgically bonded in conventional manner to an intermediate or core layer of metal 38 substantially throughout the interfaces 40 and 42 between the metal layers. More specifically, the metal layer 34 is formed of an iron alloy having a nominal composition by weight of about 22 percent nickel, 3 percent chromium and the balance iron and having a relatively high coefficient of thermal expansion of about  $10.5 \times 10^{-6}$  inches 50 55 60 65 66

per inch per degree Fahrenheit; the metal layer 36 is formed of an iron alloy having a nominal composition by weight of about 36 percent nickel and the balance iron and having a relatively low coefficient of thermal expansion of about  $0.7 \times 10^{-6}$  inches per inch per degree Fahrenheit; and the metal layer 38 is formed of a stainless steel material having a nominal composition by weight of 0.05 percent (max.) carbon, 1.00 percent (max.) manganese, 1.00 percent (max.) silicon, 10.00 to 12.00 percent chromium, 0.50 percent titanium, and the balance iron and an intermediate coefficient of thermal expansion of about  $6.0 \times 10^{-6}$  inches per inch per degree Fahrenheit. Alternately, the metal layer 38 is formed of a stainless steel of comparable thermal expansion properties such as an alloy having a nominal composition, by weight, of 0.08 percent (max.) carbon, 1.00 percent (max.) manganese, 1.00 percent (max.) silicon, 0.030 percent (max.) sulfur, 11.50 to 14.50 percent chromium, 0.10 to 0.30 percent aluminum and the balance iron or an alloy having a nominal composition, by weight, of 0.15 percent (max.) carbon, 1.00 percent (max.) manganese, 1.00 percent (max.) silicon, 0.030 percent (max.) sulfur, 11.50 to 13.50 percent chromium, and the balance iron. Most importantly, in the thermostat material of this invention, the metal layers 34 and 36 each have approximately the same thickness comprising from about 17.5 to 27.5 percent of the total thickness of the composite material and the metal layer 38 has a thickness comprising about 45 to 65 percent of the total thickness of the composite thermostat material.

In this arrangement, the thermostat metal material embodied in the support members 24 is entirely formed from iron alloy materials which do not tend to contaminate the atmosphere or the phosphors in the tube 10; the metals embodied in the support each display substantial strength at the elevated temperatures up to about 350°F. to which they will be subjected in the tube 10; the metals in the outer layers 34 and 36 of the thermostat metal supports comprise the materials conventionally used in shadow mask supports in color television tubes other than those of slim design and are therefore known and accepted in the market place as being free of contaminating effects and as providing stable thermal response characteristics over a long cycle life; the metal of the layer 38 in the support members 24 is of relatively low cost; and most important, use of the relatively very thick core layer 38 in the thermostat material of this invention provides the thermostat material embodied in the supports 24 with relatively low flexibility (as defined by the American Society for Testing Metals) in the range from 90 to 110 at temperatures up to 350°F. The use of the relatively thick layer 38 of a relatively very inexpensive metal material also significantly reduces the cost of the thermostat metal. Accordingly, the thermostat metal support members 24 are easily proportioned for moving the shadow mask 22 toward the tube face 16 as the tube 10 becomes heated during operation, thereby to compensate for the thermal expansion of the mask 22 to retain the mask aper-

tures in registry with the respective phosphors 18 on the tube face during such tube operation in conventional manner.

Preferably, for example, in a preferred embodiment of this invention, each of the supports 24 is formed of thermostat metal material having a thickness of about 0.030 to 0.050 inches wherein the core layer 38 of the thermostat material comprises about 55 percent of the total thickness of the thermostat metal and provides the thermostat metal with the desired combination of properties including a low flexibility of about 100 at temperatures up to about 350°F.

It should be understood that the embodiments of the thermostat metal material and the shadow mask support arrangement which have been described above have been described by way of illustrating this invention and that this invention includes all modifications and equivalents of the described embodiments falling within the scope of the appended claims.

I claim:

1. In a slim color television tube having a tube envelope with a tube face and phosphors disposed on the tube face and having a shadow mask with a multiplicity of apertures therein arranged with the mask apertures in registry with respective phosphors on the tube face, means supporting the mask on the tube envelope compensating for thermal expansion of the mask to retain the mask apertures in registry with the respective phosphors during heating of the mask, said support means being formed of a composite thermostat metal having an outer layer of selected thickness of a metal alloy having a nominal composition by weight of about 22 percent nickel, 3 percent chromium and the balance iron, another outer layer of approximately equal thickness of a metal alloy having a nominal composition by weight of about 36 percent nickel and the balance iron, and an intermediate layer of a metal alloy selected from the group consisting of an alloy having a nominal composition by weight of 0.05 percent (max.) carbon, 1.00 percent (max.) manganese, 1.00 percent (max.) silicon, 10.00 to 12.00 percent chromium, 0.50 percent titanium, and the balance iron, an alloy having a nominal composition by weight of 0.08 percent (max.) carbon, 1.00 percent (max.) manganese, 1.00 percent (max.) silicon, 0.030 percent (max.) sulfur, 11.50 to 14.50 percent chromium, 0.10 to 0.30 percent aluminum and the balance iron, and an alloy having a nominal composition by weight of 0.15 percent (max.) carbon, 1.00 percent (max.) manganese, 1.00 percent (max.) silicon, 0.030 percent (max.) sulfur, 11.50 to 13.50 percent chromium, and the balance iron, said intermediate metal layer being disposed between and metallurgically bonded to said outer metal layers and having a thickness comprising from about 45 to 65 percent of the total thickness of the composite material providing the composite material with a flexibility of about 90 to 110 in the temperature range from room temperature up to about 350°F.

\* \* \* \* \*